

Oct. 4, 1966

R. S. SERY ET AL  
METHOD OF PRODUCING MAGNETIC CORES BY USING  
ELECTRON IRRADIATION  
Filed April 28, 1964

3,276,922



Robert S. Sery & Daniel I. Gordon  
INVENTORS.

BY

*W. J. Griswold*  
ATTORNEY.  
*Roger J. Erickson*  
AGENT.

3,276,922

METHOD OF PRODUCING MAGNETIC CORES BY  
USING ELECTRON IRRADIATION

Robert S. Sery, Silver Spring, and Daniel I. Gordon, Chevy Chase, Md., assignors to the United States of America as represented by the Secretary of the Navy

Filed Apr. 28, 1964, Ser. No. 363,310

5 Claims. (Cl. 148—100)

The invention described herein may be manufactured and used by or for the Government of the United States of America for governmental purposes without the payment of any royalties thereon or therefor.

The present invention relates to the method of treating materials of high magnetic permeability in such a way as to impart to said materials the characteristic of exhibiting a tri-stable hysteresis loop.

Magnetic materials have extensive use in present day technology, and in some applications such as computer logic circuitry where three memory states are needed, for example, it is desirable that these magnetic materials exhibit the characteristic of having tri-stable hysteresis loops. In the past, the only processes known for imparting such characteristics to a magnetic material have been high temperature annealing processes, which require that the magnetic material be subjected to temperatures in the order of 490° C. to 1000° C. for periods of time exceeding 20 hours. Unlike the prior methods which were extremely cumbersome and time consuming, the present invention produces magnetic materials having tri-stable hysteresis loops by intermittently irradiating the material with electrons while maintaining the temperature below those conventionally used for thermal annealing.

It is an object of this invention to provide a new method of treating materials of high magnetic permeability to cause the materials to exhibit tri-stable hysteresis loops.

Another object of the invention is to provide a safe, fast, and reliable method of treating materials of high magnetic permeability to exhibit hysteresis loops which have three levels of stability.

The figure of the drawing illustrates a graph which shows the hysteresis loops of a particular material both before and after being treated according to the method of the present invention.

In the practice of this invention, flat core materials are irradiated with electrons from a suitable electron source, such as a Van de Graaf accelerator, for example, while maintaining the temperature of the core materials generally low with respect to the ordering temperature of the material, i.e. maintaining the temperature of the material below that temperature at which permanent heat treatments are produced. The irradiation of the core material is administered in three separate intermittent stages or doses, each dose being separated by an interval of time during which no irradiation is directed upon the core material. It has been found that an electron beam having a sufficiently high energy level will, when directed upon a flat core material, alter the magnetic properties of said material. As a result of this process, it is believed that certain of the atoms in the molecular lattice of the core material are displaced from their normal positions when bombarded by electrons, thus producing interstitial atoms and vacancies, which thereby change the ordering of the material and impart to the material different magnetic characteristics, as evidenced by a change in the shape of its hysteresis loop. It is believed that an electron beam as low as 0.5 m.e.v. will produce this effect and it has been found, for example, that electrons at 2 m.e.v. will definitely be sufficient to produce said effect.

By way of example, a punched ring of 4.75% Mo Permalloy (4.75% molybdenum, 79% nickel, and 16.25%

iron) was treated according to the method of this invention in the following manner:

A punched ring of 4.75% Mo Permalloy which had been heat treated for high permeability and having an inner diameter of  $\frac{5}{8}$  inch and an outer diameter of  $1\frac{3}{16}$  inch and being .006 inch in thickness was irradiated with a 2 m.e.v. electron beam. A Van de Graaf accelerator was used as the electron source and the ring was supported by an electrically conductive block which was electrically grounded to serve as an electron collector during the irradiation. The block had internal passages formed therein to permit the flow of a coolant therethrough and thus provided means to maintain the temperature of the ring material substantially below its ordering temperature. The ring or core material was irradiated with the electron beam for a period of 15 minutes, the Van de Graaf accelerator was then shut down for a period of 15 minutes, the core material was again irradiated by the electron beam for a second period of 15 minutes, followed by a second shut down period of 20 minutes duration. The Van de Graaf accelerator was then reactivated for an additional period of 65 minutes, thus completing the treatment. During this process, the temperature of the core material ranged from 90° C. at the beginning of the irradiation to a high of 134° C. at the end of the irradiation. The electron flux was

$$1.13 \times 10^{18} \frac{e/cm.^2}{min.}$$

30 and the total or integrated electron flux was  $1.1 \times 10^{17}$  electrons/cm.<sup>2</sup>.

Referring to the figure of the drawings, wherein the hysteresis loop for the ring measured prior to the treatment in the matter of the present invention is shown in dotted line form while the ring's hysteresis loop measured after said treatment is shown in solid line form, it may clearly be seen that the magnetic properties of the core material have been appreciably altered by the method of this invention and that the material now exhibits a hysteresis loop which has three distinct levels of stability, i.e. three distinct levels of magnetic induction. The number of doses or periods of irradiation are not determinative of the number of saturation levels exhibited by the core material; but rather, only one additional saturation level is induced in the material when said material is intermittently irradiated by an electron beam of proper dose and sufficient energy. The method of the present invention therefore clearly alters the conventional shape of the hysteresis loop of the core material and its magnetic characteristics and renders that material ideally suitable for certain applications wherein tri-stable core materials are needed in modern ferro-resonant circuits.

The method described above is intended to be no more than an example and is not intended to restrict the invention to the values and ranges specified. Some of the factors which may selectively vary to change the resultant characteristics of the cores treated according to the method of this invention are the energy level of the electron beam, the current of the electron beam, the total integrated electron flux, the temperatures of the core materials, the core material, the dimensions of the core materials, the type of atomic particles used to bombard the core material, and the time durations of irradiation and time durations of rest.

65 The above method quickly, reliably, and safely produces magnetic cores which are not radioactive and which have tri-stable hysteresis loops from conventional magnetic materials having high magnetic permeability.

Obviously many modifications and variations of the present invention are possible in light of the above teachings. It is therefore to be understood that within the

scope of the appended claims the invention may be practiced otherwise than as specifically described.

What is claimed is:

1. A method of changing the magnetic properties of a material comprising the steps of

intermittently directing a beam of high energy atomic particles onto the material for collision therewith for predetermined durations of time, whereby the number of levels of magnetic stability is increased.

2. A method of treating a material having a high magnetic permeability to cause the material to exhibit a tri-stable hysteresis loop comprising the steps of

irradiating the material with a beam of electrons of energies greater than 0.5 m.e.v. for a plurality of intermittent predetermined intervals of time, the successive intervals being separated by predetermined periods of time during which the material is protected from the electrons.

3. A method of treating a material of high magnetic permeability to cause the material to exhibit a tri-stable hysteresis loop comprising the steps of

directing an intermittent beam of electrons of energies in excess of 0.5 m.e.v. onto a material of high magnetic permeability, and cooling the material to maintain the temperature of the material below its conventional heat treatment temperature.

4. A method of treating a flat core of a nickel-iron alloy having high magnetic permeability comprising the steps of

irradiating the core with an intermittent beam of high energy atomic particles having an energy level greater than 0.5 m.e.v. for a plurality of predetermined periods of time,

protecting the core from irradiation for preselected intervals of time between said periods of irradiation, and

cooling the core during the periods of irradiation to maintain the temperature of the core below 250° C.,

whereby the core is caused to exhibit a tri-stable hysteresis loop.

5. A method of changing the magnetic properties of a nickel-iron alloy of high magnetic permeability comprising the steps of

irradiating the alloy with an electron beam of an energy level of approximately 2 m.e.v. for approximately fifteen minutes,

protecting the alloy from irradiation for approximately fifteen minutes,

irradiating the alloy with the electron beam for approximately fifteen minutes,

protecting the alloy from irradiation for twenty minutes,

irradiating the alloy with the electron beam for approximately sixty five minutes, and

cooling the alloy during each period of irradiation to maintain the temperature of the material below its ordering temperature,

whereby the alloy is caused to exhibit a tri-stable hysteresis loop.

#### References Cited by the Examiner

##### UNITED STATES PATENTS

2,968,723 1/1961 Steigerwald \_\_\_\_\_ 148—1.5  
3,192,078 6/1965 Gordon et al. \_\_\_\_\_ 148—100

##### OTHER REFERENCES

Gordon et al.: Article in Solid State Physics in Electronics and Telecommunications, vol. 4, pp. 824—858, Sept. 1, 1960.

Seitz et al.: Article in Solid State Physics, vol. 2, pp. 305—448, June 1956.

Sery et al.: Article in Journal of Applied Physics, vol. 34, pp. 1311—1312, April 1963.

DAVID L. RECK, *Primary Examiner*.

N. F. MARKVA, *Assistant Examiner*.